

March 6, 1945.

J. E. HAZELTINE, JR

2,371,049

BUILDING STRUCTURE

Filed Aug. 6, 1941

*Fig. 1*



*Fig. 2*



*Fig. 3*



Inventor  
James E. Hazeltine, Jr.  
by  
Walter J. Kugman

Attorney

## UNITED STATES PATENT OFFICE

2,371,049

## BUILDING STRUCTURE

James E. Hazeltine, Jr., Lancaster, Pa., assignor  
to Armstrong Cork Company, Lancaster, Pa.,  
a corporation of Pennsylvania

Application August 6, 1941, Serial No. 405,681

9 Claims. (Cl. 154—49)

This invention is particularly concerned with floors or walls covered with a material having a body or foundation made of waterproof impregnated fibrous material. Typical coverings of this sort are known as felt base and felt backed linoleum and comprise a foundation of asphalt impregnated felt and a wearing layer of oil paint in the case of felt base or linoleum composition in felt backed linoleum. The underside of such coverings is provided with a paint coating which usually serves the dual purpose of concealing the unsightly asphalt saturant of the felt and at the same time sealing it against bleeding onto the face of the material when it is rolled for storage and shipment.

Felt base floor coverings have generally been laid loose on the floor rather than cemented, because of the impossibility of removing them when so cemented. The felt body is inherently weak and ruptures when any attempt is made to strip it from the floor. This condition is aggravated by the generally laminar character of the felt, due to the felting operation in its formation, for the felt tends to pull apart at different levels between its top and bottom surfaces, leaving an irregular layer of asphalt saturated felt attached to the floor, which cannot for all practical purposes be successfully removed.

This problem has been recognized for the advantages of permanently cementing the floor covering in place are important. In recent years, there has been introduced on the market, felt base materials which may be satisfactorily cemented in place. Cementing is desirable since it prevents any substantial expansion of the covering which results in buckling and consequent breakage, and at the same time, it eliminates the use of unsightly and hazardous metal binding strips over the seams. Wall coverings must be cemented in place.

There are two types of felt base floor coverings now in common use which may be cemented in place and subsequently removed from the floor.

In one type, removability of the covering is attained by the use of a permanently plastic layer of rubber disposed between the felt base and the adhesive used to secure the covering to the floor. The permanently plastic material has greater affinity for the felt than it has for the adhesive and as a consequence it breaks away from the adhesive when removal of the covering is effected.

In the second type, a coating is applied to the underside of the felt base and this coating has the characteristic of parting or rupturing internally. Its resistance to rupture is less than the felt base to which it is applied. In the application of this material, a layer of adhesive is applied to the floor and the material is pressed into engagement with it. The partible coating is thus disposed between the felt base and the

adhesive and constitutes a weak link in the structure. When it is desired to remove the covering, it is pried loose in one corner of the room and is stripped from the floor by rupture of the partible coating. This is possible because the partible coating is materially weaker than the felt base and the coating ruptures internally before the felt tears.

My invention relates to an improvement in the structure of the latter class, that is, those in which a partible coating is employed.

In the manufacture of such floor coverings, it has been found necessary to formulate the partible coatings specifically for each type of material to which such coatings were to be applied, because difference in the time and temperature of the curing of the material altered the characteristics of rupturability or partibility of the coatings. The range of rupturability of the partible coating is not too wide and it is desirable to be able to produce material having a coating falling within a rather restricted range.

It has heretofore been determined that there are certain limits of cohesion, within which the required rupturability of the partible coating is obtained. Limits of 3 to 30 pounds resistance are satisfactory, but limits of 6 to 30 pounds are preferred. If the tensile resistance be substantially greater than 30 pounds, the rupturable coating is so strong as to prevent ready removability, and with tensile resistance substantially less than 3 pounds, there is some danger of the covering becoming loose during use, due to heavy traffic conditions. For that reason, a minimum of 6 pounds is preferred. Felt base products have a tensile strength above 30 pounds in that samples do not rupture when attempts are made to remove them from blocks of wood with an interposed partible coating which ruptures at 30 pounds.

The limits of cohesion may be determined by the Scott test in the following manner:

To one side of a strip of wood 6 inches long by 2 inches wide a thin layer of linoleum cement or paste is applied, using a notched doctor blade to distribute the paste or cement evenly over the entire surface. To the paste or cement is immediately applied a strip of the covering to be tested 8 inches by 2 inches wide, one end of which is placed flush with one end of the strip of wood, the other end extending free beyond the wood strip. After rolling to obtain a satisfactory bond between the wood and the covering, the sample is maintained at normal room temperature for approximately four days to dry the paste or cement. The resistance of the coating to tensile forces is determined by placing the sample in a Scott tensile strength machine at right angles to the direction of the forces to be exerted. The strength of the forces recorded as the covering is removed from the wood strip

measures the resistance of the coating to tensile forces.

As an example of the problem involved in floor covering manufacture, the partible coating for use on Linoflor, where the wearing surface is a linoleum composition, which is stoved for a relatively long period of time, say 10 days, and at relatively high temperatures, say 190° F., must be formulated differently than a similar coating for use on printed felt base where the wear layer is an oil paint, which is cured or set by stoving for a relatively shorter time and at relatively lower temperatures. Thus, each time the formulation of the wearing surface is materially changed, it is necessary to reformulate the coating in order to obtain rupturability within the desired range. Any substantial increase in the temperature of stoving or curing, due to changes in the formulation of the paint or linoleum composition requiring higher temperatures for best results, necessitates a reformulation of the partible coating to obtain partibility within the range desired for optimum results. Accidental overheating in stoving sometimes results in complete failure of the partible coating.

Many experiments have been conducted to find a satisfactory solution to this problem and great effort has been expended to find a universal coating possessing the requisite rupturability. The general belief has been that the heating in the curing stoves or ovens for setting the paint or maturing the linoleum composition has induced some chemical reaction in the rupturable coating, increasing its strength to the point where it will not rupture prior to tearing of the felt. This is a logical theory and has been extensively explored. I have now discovered, however, that the deleterious action caused by heat is apparently due to some slight permeation of the asphalt saturant of the felt base into the rupturable coating, for I have found that by providing a coating directly on the felt base, which is a positive barrier to the migration or bleeding of the asphalt therethrough and applying the rupturable coating to the barrier coating, time and temperature conditions no longer materially affect the rupturable coating. The same rupturable coating may now be used on printed felt base as is used on Linoflor. The problems of overheating or changes in formulation of the wearing surface of the covering, which previously required the formulation of new rupturable coatings, are completely eliminated.

According to the present invention, I provide a coating on the under surface of the saturated felt base or foundation, and this coating is so formulated as to act as a positive barrier against the bleeding of the asphalt impregnant therethrough. To this layer I apply a rupturable coating and, if desired, the rupturable coating may be covered with one or more coats of oil or casein paint, or the like, to give the under surface of the product a pleasing appearance while on display.

The following example will illustrate my invention. It should be understood that it is not limited to any particular ingredients, either in the seal coat or rupturable coat or, in fact, in the decorative coat. Each must produce a certain result and the physical characteristics of each coating are availed of to produce that result—the seal coat must be a positive barrier to the migration of the asphalt or other saturant of the felt base; the partible coating must be materially weaker than the felt base so as to rupture in-

ternally before the felt tears; and the decorative paint should present a pleasing appearance. Many different coatings will be found to possess the required characteristics. My invention is not in the coatings themselves but the covering and the building structure including the covering cemented in place.

Referring to the drawing, there is shown:

10 In Figure 1 a sectional view of a floor or wall covering embodying my invention;

In Figure 2 a perspective view, broken away, illustrating a modification of my invention; and

15 In Figure 3 an enlarged view of a building structure embodying my invention, showing the covering of Figure 1 secured in place by an adhesive.

The covering shown in Figure 1 comprises a linoleum composition wear layer 2, an asphalt saturated base or foundation 3, a barrier coating 4, a partible coating 5, and a decorative paint 6.

20 As heretofore pointed out, the essential characteristic of the coating 4 is that it act as a positive barrier to the migration or bleeding of the asphalt or other saturant from the felt base layer 3. The coating 4 may be formulated as follows:

|                   | Parts by weight |
|-------------------|-----------------|
| Casein            | 60.00           |
| Ammonia 26° Baume | 6.00            |
| Formalin          | 4.60            |
| Water             | 492.00          |

30 In this coating, the casein is the binder. Ammonia is used as an alkali to render the casein soluble. Formalin is used as an insolubilizing agent for the casein and water is a vehicle. The particular formulation of the seal coating is not important, provided it act as a barrier to the saturant of the felt base.

35 The partible coating 5 may be formulated as follows:

|                       | Parts by weight |
|-----------------------|-----------------|
| Soy bean protein      | 35.00           |
| Borax                 | 7.50            |
| Formalin              | 3.00            |
| 45 No. 3 refined clay | 466.00          |
| Water                 | 538.00          |

45 In this coating, the soy bean protein is the binder and borax is an alkali serving to render the protein water soluble. The formalin and water serve purposes similar to those served in the seal coat above referred to. The refined clay in the rupturable or partible coating is a filler. The particular ingredients used in the rupturable coating are not important, so long as they produce a final coating which is materially weaker than the felt base in resistance to rupture, preferably in the range of 6 to 30 pounds, as determined by the Scott test.

50 The decorative paint is used to enhance the appearance of the product when exhibited for sale. A typical formula for this paint may be as follows:

|                       | Parts by weight |
|-----------------------|-----------------|
| 65 Casein             | 52.50           |
| Borax                 | 7.00            |
| Sodium metasilicate   | .63             |
| Formalin              | 4.00            |
| 70 No. 3 refined clay | 392.00          |
| Red pigment           | 39.00           |
| Whiting               | 87.50           |
| Water                 | 556.00          |

75 In Figure 2, I have shown a modified floor covering in which there are provided two thicknesses of paint 6 and 7, which serve as decora-

tive coatings for the back surface of the felt. These layers may be of the decorative coating above referred to, applied in two coats, or one coat may be more or less of a size coat and a final coat pigmented to the desired color.

Figure 3 illustrates a typical building structure embodying my invention. The floor covering of Figure 1 is secured by means of an adhesive 8 to a floor or wall surface 9. The enlarged portion of Figure 3 diagrammatically illustrates removal of the covering by rupture of the coating 5. It will be seen that when the covering is stripped from the area to which it is cemented, the coating 5 ruptures about midway of its thickness, permitting ready removal without damage and leaving the base in condition to receive a new covering.

From the foregoing, it will be seen that by my invention a building structure is created in which a floor covering, having a saturated felt body may be adhesively secured in permanent relationship to a floor or wall structure, and removed therefrom by rupture of a partible coating which is disposed between the saturated felt base and the floor or wall structure, the coating being materially weaker than the felt base in resistance to rupture, and to a floor or wall covering in which the rupturable coating is protected by an interposed barrier coating against deleterious attack by the saturant of the felt base.

While I have described and illustrated certain preferred embodiments in my invention, it will be understood that it is not limited to such form, since it may be otherwise embodied within the scope of the following claims.

I claim:

1. A hard surface covering including a sheet of partible fibrous material impregnated with a moisture resistant substance, a barrier coating applied to the fibrous material, and a partible coating materially weaker than the fibrous material in resistance to rupture applied over the barrier coating, the barrier coating preventing the migration of the impregnant for the fibrous material into the partible coating which would alter the strength of the partible coating in resistance to rupture.

2. A hard surface covering including a sheet of a partible fibrous material impregnated with a moisture resistant substance, a partible coating having a resistance to rupture in the range of 3 to 30 pounds determined by the "Scott test," and being materially weaker than the fibrous material applied to said sheet, and a barrier coating interposed between said sheet and said partible coating to prevent migration of the impregnant for the fibrous material into the partible coating which would alter the strength of the partible coating in resistance to rupture.

3. A hard surface covering including a sheet of partible fibrous material impregnated with a moisture resistant substance, a partible coating having a resistance to rupture in the range of 6 to 30 pounds determined by the "Scott test," and being materially weaker than the fibrous material applied to said sheet, and a barrier coating interposed between said sheet and said partible coating to prevent migration of the impregnant for the fibrous material into the partible coating which would alter the strength of the partible coating in resistance to rupture.

4. A hard surface covering including a sheet of felt impregnated with a moisture resistant substance, a barrier coating applied to the fibrous material, a partible coating materially weaker than the fibrous material in resistance to rupture applied over the barrier coating, the barrier coating preventing the migration of the impregnant for the fibrous material into the partible coating which would alter the strength of the partible coating in resistance to rupture, and a decorative paint applied over the partible coating.

5. A hard surface covering including a sheet of felt impregnated with asphalt, a partible coating, materially weaker than the felt in resistance to rupture, applied to said sheet, and a barrier coating interposed between said sheet and said partible coating to prevent migration of the impregnant for the fibrous material into the partible coating which would alter the strength of the partible coating in resistance to rupture.

6. A hard surface covering including a sheet of partible fibrous material impregnated with a moisture resistant substance, a barrier coating applied to the fibrous material, and a partible coating materially weaker than the fibrous material in resistance to rupture applied over the barrier coating, the barrier coating preventing any heat induced migration of the impregnant for the fibrous material into the partible coating which would alter the strength of the coating in resistance to rupture whereby the temperature at which the covering is heated in the curing thereof does not affect the rupturable characteristics of the partible coating.

7. A hard surface covering including a sheet of asphalt impregnated felt, a partible coating materially weaker than the felt in resistance to rupture applied to said sheet, and a barrier coating including casein interposed between said sheet and said partible coating to prevent migration of the impregnant for the fibrous material into the partible coating which would alter the strength of the partible coating in resistance to rupture.

8. A hard surface covering including a sheet of partible fibrous material impregnated with asphalt, a partible coating having a resistance to rupture in the range of 3 to 30 pounds determined by the "Scott test," and being materially weaker than the fibrous material in resistance to rupture applied to said sheet, and a barrier coating interposed between said sheet and said partible coating to prevent migration of the asphalt impregnant for the fibrous material into the partible coating which would alter the strength of the partible coating in resistance to rupture.

9. A hard surface covering including a sheet of felt impregnated with asphalt, a partible coating having a resistance to rupture in the range of 6 to 30 pounds determined by the "Scott test," and being materially weaker than the fibrous material in resistance to rupture applied to said sheet, a barrier coating interposed between said sheet and said partible coating to prevent migration of the asphalt impregnant for the fibrous material into the partible coating which would alter the strength of the partible coating in resistance to rupture, and a wear layer applied to the opposite face of said sheet.

JAMES E. HAZELTINE, JR.